

Nov. 13, 1923.

M. BROWN

1,473,695

INNERSOLE

Filed June 10, 1921



Inventor:  
Max Brown  
by Clyde L. Rogers  
his Atty.

## UNITED STATES PATENT OFFICE.

MAX BROWN, OF BOSTON, MASSACHUSETTS.

## INNERSOLE.

Application filed June 10, 1921. Serial No. 476,465.

*To all whom it may concern:*

Be it known that I, MAX BROWN, a citizen of the United States, and resident of Boston, county of Suffolk, Commonwealth of Massachusetts, have invented an Improvement in Innersoles, of which the following description, in connection with the accompanying drawings, is a specification, like characters on the drawings representing like parts in each of the several views.

This invention relates to innersoles of shoes and boots and more particularly to an improved composite innersole produced of a plurality of layers of specially selected materials. A principal object of the invention is to provide an innersole that exhibits qualities of strength and insulation against moisture and cold in a high degree while being inexpensive and produced throughout of materials easily and cheaply obtained. The foregoing and other objects and advantages of the invention will more fully appear from the following detailed description, and the distinctive features of novelty will be pointed out in the appended claims.

Referring to the drawings:

Figure 1 is an elevation of an innersole embodying the invention with portions of the successive layers broken away to better show the interior construction;

Fig. 2 is an edge view thereof; and

Fig. 3 is an elevation of the innersole.

In carrying out the invention I provide two layers 10, 11, of a light or medium weight felt, preferably about a twenty pound grade. These felt layers are saturated with asphaltum or a like waterproof cementitious binder and they are pressed together with an intermediate layer 12 of stout burlap, the asphaltic coating of the felt layers uniting firmly and strongly with the fibres of the burlap. To the outer side of the burlap layer 10 is applied a layer 13 of paper preferably of a stout grade such as kraft paper. This constitutes the outer side of the innersole. To the surface of the felt layer 11 a fleece lining layer 14 may be applied. These layers when united and pressed together are all held strongly by the adhesive bond of the

asphalt with which the felt layers 10, 11, are loaded, so that the innersole thus produced is a unitary mass, the several layers or laminæ of which are strongly adherent. Among the advantages of the composite innersole thus produced, are that the burlap with its stout crisscross threads imparts strength to hold the stitching in the assembling of the innersole, while the felt layers provide insulation against heat and cold, and the asphalt serves the double purpose of a cementitious binder and of providing complete insulation against moisture. The outer paper layer 13 protects the outer surface of the felt layer 10, and together with the fleece lining 14 applied to the layer 11, prevents any exposure of the asphalt coating as the innersoles are handled in the shoe shop. I am aware that the invention may be embodied in other specific forms without departing from the spirit or essential attributes thereof, and I therefore desire the present embodiment to be considered in all respects as illustrative and not restrictive, reference being had to the appended claims rather than to the foregoing description to indicate the scope of the invention.

Having described my invention, what I claim as new and desire to secure by Letters Patent is:

1. An innersole comprising two asphalt-saturated layers of felt adhesively secured together with an intermediate layer of burlap, to constitute a composite unitary innersole.

2. An innersole comprising two felt layers loaded with waterproof cementitious binder and adhesively secured thereby with an intermediate layer of strength giving burlap or the like.

3. An innersole comprising a plurality of layers of felt loaded with waterproof cementitious binder adhesively secured with an intermediate layer of strength giving burlap, and with protective layers applied to the outer surfaces of said felt layers.

In testimony whereof, I have signed my name to this specification.

MAX BROWN.